

# United States Patent

[11] 3,634,211

[72] Inventor Edgar J. Seyb, Jr.  
Oak Park, Mich.  
[21] Appl. No. 864,170  
[22] Filed Oct. 6, 1969  
[45] Patented Jan. 11, 1972  
[73] Assignee M & T Chemicals Inc.  
New York, N.Y.

[54] **PROCESS FOR ELECTROPLATING CHROMIUM  
AND ELECTROLYTES THEREFOR**  
13 Claims, No Drawings

[52] U.S. Cl. .... 204/51  
[51] Int. Cl. .... C23b 5/06  
[50] Field of Search. .... 204/51,  
Machine Searched

[56] **References Cited**  
UNITED STATES PATENTS  
3,334,033 8/1967 Romanowski et al. .... 204/51

*Primary Examiner—G. L. Kaplan*  
*Attorneys—Lewis C. Brown, Kenneth G. Wheeless and Robert*  
*P. Grindle*

**ABSTRACT:** In accordance with certain of its aspects, this invention relates to novel compositions and to a process for electroplating chromium plate onto a basis metal which comprises passing current from an anode to a cathode at least a portion of which contains a conductive metal layer through an aqueous acidic chromium-plating solution substantially free of nitric acid and other oxidative catalysts containing

1. at least one chromium compound providing hexavalent chromium ions for electroplating chromium; and
2. cerous ions in combination with fluoride ions and sulfate ions as catalysts;

for a time sufficient to deposit a chromium electroplate having a thickness of at least  $1 \times 10^{-4}$  mm.

## PROCESS FOR ELECTROPLATING CHROMIUM AND ELECTROLYTES THEREFOR

This invention relates to novel compositions and to novel processes for the electrodeposition of chromium from an aqueous acidic chromium-plating bath.

It is known that chromium may be plated onto various basis metals from aqueous bath solutions. During chromium plating using such bath compositions it has been found that the use of certain catalysts such as silicofluoride ions and sulfate ions provide improved chromium electrodeposits especially in so-called low current density areas. The effect of such catalyst systems, however, has been found to vary with the concentration of the chromic acid and the ratio of the catalysts to the total chromic acid content. Since the concentration of the chromium-plating bath continually varies during operation due to the removal of chromium in the form of deposited metal and due to the addition of impurities arising from the electrodes as well as decomposition products, it has been difficult to control and maintain the proper catalyst and chromic acid concentrations throughout the life of a typical aqueous acidic chromium-electroplating bath.

It has now been found that the addition of cerous ions in combination with fluoride and sulfate catalyst ions in an aqueous acidic bath containing chromic acid results in a chromium-electroplating composition which is stable over the life of the bath and maintains the activity of the bath over its useful life by regulating the concentrations of the catalyst ions as the chromic acid concentration is depleted and in the presence of typical impurities and decomposition products which occur during the chromium-plating operation.

It is an object of this invention to provide improved electroplating compositions and processes. A further object of the invention is to provide stabilized chromium-plating bath compositions which have good throwing power and extended useful life. Other object of the invention will be apparent to those skilled in the art upon inspection of the following detailed description of the invention.

In accordance with certain of its aspects, this invention relates to novel compositions and to a process for electroplating chromium plate onto a basis metal which comprises passing current from an anode to a cathode at least a portion of which contains a conductive metal layer through an aqueous acidic chromium-plating solution substantially free of nitric acid and other oxidative catalysts containing

1. at least one chromium compound providing hexavalent chromium ions for electroplating chromium; and
2. cerous ions in combination with fluoride ions and sulfate ions as catalysts;

for a time sufficient to deposit a chromium electroplate having a thickness of at least  $1 \times 10^{-4}$  mm.

The chromium electroplating bath compositions of the invention may contain about 100-600 g./l. of chromic acid (expressed as  $\text{CrO}_3$ , and preferably about 200-350 g./l. of chromic acid. The fluoride ions may be added to the chromium electroplating bath in the form of compounds such as sodium silicofluoride ( $\text{Na}_2\text{SiF}_6$ ), fluosilicic acid ( $\text{H}_2\text{SiF}_6$ ), strontium silicofluoride ( $\text{SrSiF}_6$ ), ammonium silicofluoride [ $(\text{NH}_4)_2\text{SiF}_6$ ], magnesium silicofluoride ( $\text{MgSiF}_6$ ), calcium silicofluoride ( $\text{CaSiF}_6$ ), etc. Other fluoride compounds which may be used in the bath according to the invention include sodium fluoride, potassium fluoride, calcium fluoride, hydrofluoric acid, ceric fluoride, cerous fluoride, etc. Other fluoride ions (including complex fluoride ions) which may be employed include, for example, fluoaluminates, fluoborates, fluotitanates, and fluozirconates.

The sulfate ions may be added to the chromium-electroplating bath in the form of suitable sulfate compounds such as strontium sulfate ( $\text{SrSO}_4$ ); sulfuric acid ( $\text{H}_2\text{SO}_4$ ); lithium sulfate ( $\text{Li}_2\text{SO}_4$ ); ammonium sulfate [ $(\text{NH}_4)_2\text{SO}_4$ ]; calcium sulfate ( $\text{CaSO}_4$ ); etc.

The chromium electroplating process may use temperatures of 30°-70° C. with a chromic acid bath containing 100-600 g./l. of chromic acid (as  $\text{CrO}_3$ ). The ratio of chromic acid to

sulfate ion ( $\text{CrO}_3:\text{SO}_4^{2-}$ ) may be maintained at 100-500:1, typically 150-300:1 and preferably about 200:1.

Cerous ions may be added to the bath in the form of salts such as cerium carbonate, cerium fluoride, cerium sulfate, etc. 5 When cerium fluoride ( $\text{CeF}_3$ ) is employed in combination with fluoride, fluoride-containing and/or sulfate catalysts, the chromium plating bath composition (containing 100-600 g./l. of  $\text{CrO}_3$ ) may be saturated with  $\text{CeF}_3$ . Such saturation is provided to obtain self-regulation of the catalyst content of the bath. Typically, from about 1 to 4 g./l. or more of  $\text{CeF}_3$  (or other cerous salts including complex fluoride salts) may be added to a chromium plating solution containing 100-600 g./l.  $\text{CrO}_3$  to form a chromic acid solution which contains excess undissolved cerium fluoride ( $\text{CeF}_3$ ). Excess cerous ion concentrations derived from other cerium salts may be utilized to suppress and further control the fluoride ion concentration.

Quite unexpectedly and of great advantage is the fact that, unlike other proposed sparingly soluble catalyst control materials, the solubility of the cerous fluoride is virtually independent of the temperature of the solution in the range of most interest during plating when compared with other sparingly soluble fluoride compounds which have been found to have an appreciable temperature coefficient of solubility. In 20 practice this means that when use of these materials as catalyst regulators is attempted, more of the material is dissolved at the higher (operating) temperatures and appreciable material precipitates out when the solution is allowed to cool, e.g. due to a process shutdown or routine overnight or weekend interruption.

On startup, when such solution is first reheated, the proper concentration of catalyst may not be attained for some time so that plating may not be immediately started. The remarkable 25 constancy of solubility of the cerous fluoride as employed in the invention herein makes it possible to initiate plating as soon as the solution reaches operating temperature.

These same considerations lead to other significant practical advantages. For example, other previous so-called self-regulated baths may need extensive agitation to aid in solution 30 of the catalytic material during reheat. The new baths employed according to the invention herein may obviate the need for excessive agitation for this purpose because the proper amount of required catalyst is already dissolved.

Although chromic acid concentration of less than 100-600 g./l. may be used, the preferred range is 100-600 g./l., and the most preferred range is 200-400 g./l.

In general, as the chromic acid concentration increases, so does the equilibrium solubility of the fluoride ion. There are at 35 least two beneficial results from this fact:

1. If only small changes are to be expected in normal use, the chromic acid:fluoride ratio remains relatively constant leading to uniformity of operation; and
2. Effective regulations in chromic acid:fluoride ratios can be obtained by changes in chromic acid concentration without corresponding modifications of fluoride concentration.

The concentration of the fluoride ion may be further suppressed by the use of an excess of cerous ion as supplied, for 40 example, by cerous carbonate or soluble cerous oxide.

It has further been found that in order to obtain the beneficial results of the invention herein, the cerous ion-containing baths must be essentially free of substantial quantities of oxidative catalysts (such as nitric acid, perchloric acid, etc.) to 45 prevent excessive oxidation of the cerous ion to the ceric ion on electrolysis. Because the solubility of ceric fluoride is substantially greater than the solubility of cerous fluoride, the presence of ceric ions in the bath compositions of the invention is undesirable.

70 This may be shown by the following example. Two beakers containing chromic acid, 250 g./l., and an excess of cerous fluoride were prepared. One was the control; the other was made 2.N in nitric acid. The solutions were heated to 55° C. and electrolyzed using lead anodes at 3.6 amperes for 5 hours. At this time the control solution showed the slight darkening

expected from the formation of trivalent chromium by electrolysis. The experimental solution containing the nitric acid was virtually black thus indicating that much trivalent chromium and tetravalent cerium had been formed. The oxidation was confirmed by analyzing the solutions for fluoride. The control solution contained 0.36 g./l. of fluoride. This was the amount expected from the equilibrium solubility of cerous fluoride. The experimental solution contained considerably more fluoride, 6.68 g./l. as might be expected since a substantial portion of the cerous ion had been converted to the ceric ion.

According to this invention, the aqueous acid chromium plating bath compositions of the invention may be employed at temperatures of about 30°-70° C. to prepare improved chromium plated articles by passing current from an anode to a basis metal cathode through said aqueous acidic chromium plating solution at a temperature of 30°-70° C. for a time sufficient to deposit a chromium electroplate having a thickness of at least  $1 \times 10^{-4}$  mm. Current densities which may be employed may be 1.0-90 amperes per square decimeter (asd) and preferably about 3-50 asd. The bath compositions of the invention may be used with lead anodes and/or lead alloy anodes.

The bath compositions prepared according to the invention are characterized by their excellent stability on extended use in chromium plating bath operations. In particular, the baths are characterized by excellent stability and uniformity of the fluoride: sulfate ratios in the presence of chromic acid which is saturated with cerous fluoride. The ratios have been found to remain fairly uniform over wide concentrations of chromic acid.

The following examples are submitted for the purpose of illustration only and are not to be construed as limiting the scope of the invention in any way.

The unexpectedly advantageous properties obtained by using the cerous ion in combination with fluorides (including complex fluorides) may be shown by reference to the examples summarized in table I. In each experiment, a sparingly soluble fluoride salt was formed and enough of the compound was used in the bath to provide an excess of undissolved compound. Thus, a cerous fluoride-containing precipitate remained undissolved in each solution and acted as a reservoir to control the concentration of the catalytic ion.

In each of the bath compositions described in table I, excellent chromium deposits were obtained

tivity is not directly proportional to the total fluoride because the complex fluorides may modify this activity.

The unexpected stability of operation of the plating baths of the invention may be illustrated by the use of an aqueous bath made up originally to contain 300 g./l. chromic acid, 6.6 g./l. strontium sulfate, 5.8 g./l. strontium chromate, and 3.5 cerous fluoride. The bath was allowed to equilibrate at 46° C. for three days with preelectrolysis of 4 amp-hr./liter (4 AH/L). Electrolysis was continued for a further 47 days so that the total electrolysis was 561 AH/L. Analyses at the beginning and end of electrolysis are shown in table II.

TABLE II

|                                                        |  | Example 10<br>(4.1 AH/L) | Example 16<br>(561 AH/L) |
|--------------------------------------------------------|--|--------------------------|--------------------------|
| CrO <sub>3</sub>                                       |  | 300                      | 265                      |
| SO <sub>4</sub> <sup>2-</sup>                          |  | 0.97                     | 0.88                     |
| F <sup>-</sup>                                         |  | 0.27                     | 0.28                     |
| Ratio, CrO <sub>3</sub> :SO <sub>4</sub> <sup>2-</sup> |  | 309/1                    | 301/1                    |

Electroplating was satisfactory and of substantially uniform quality throughout this period. Plating tests were completed using standard test strips in a Hull Cell. Chromium coverage was measured by plating at 2 amperes for 3 minutes at 46° C. The coverage results in mm. of chromium measured from the high current density end of the test panels are shown in table III.

TABLE III

|    | Example No. | Days | AH/LITER | Coverage (mm.) |
|----|-------------|------|----------|----------------|
| 10 | 0           |      | 4.1      | 51             |
| 11 | 1           |      | 16.3     | 52             |
| 12 | 5           |      | 34.1     | 52             |
| 13 | 8           |      | 97.5     | 51             |
| 14 | 13          |      | 168.0    | 50             |
| 15 | 21          |      | 325.0    | 50             |
| 16 | 47          |      | 561.0    | 50             |

Tables II and III clearly demonstrate that the bath compositions of the invention are remarkably and unexpectedly stable

TABLE I.—TOTAL AMOUNT OF MATERIAL IN G./L. USED FOR MAKE-UP OF THE PLATING SOLUTION

| Ingredient                                                | Example numbers |       |       |       |       |       |       |       |       |
|-----------------------------------------------------------|-----------------|-------|-------|-------|-------|-------|-------|-------|-------|
|                                                           | (1)             | (2)   | (3)   | (4)   | (5)   | (6)   | (7)   | (8)   | (9)   |
| Chromic acid                                              | 250             | 250   | 250   | 250   | 375   | 375   | 250   | 375   | 175   |
| Cerium (cerous) catalyst:                                 |                 |       |       |       |       |       |       |       |       |
| Cerous carbonate (pentahydrate)                           | 15.9            | 13.4  | 17.0  | 10.4  |       | 9.86  | 9.86  | 12.0  | 3.64  |
| Cerous fluoride                                           |                 |       |       |       | 3.70  | 3.70  |       |       |       |
| Sodium fluoroborate                                       | 18.9            |       |       |       |       |       |       |       |       |
| Sodium fluozirconate                                      |                 | 18.4  |       |       |       |       |       |       |       |
| Potassium fluorotitanate                                  |                 |       | 23.9  |       |       |       |       |       |       |
| Sodium fluosilicate                                       |                 |       |       | 18.9  |       |       |       |       |       |
| Sodium fluosilicate                                       |                 |       |       |       |       |       | 7.71  |       | 1.43  |
| Sodium fluoride                                           |                 |       |       |       |       |       |       |       |       |
| Sodium bifluoride                                         |                 |       |       |       |       |       |       | 4.1   |       |
| Sulfate catalyst:                                         |                 |       |       |       |       |       |       |       |       |
| Sulfuric acid (ml./l.)                                    |                 | 0.47  |       |       |       |       |       |       |       |
| Strontium sulfate                                         |                 |       |       |       |       |       |       |       |       |
| Sodium sulfate                                            | 1.63            |       | 1.63  | 0.93  | 2.89  | 2.89  | 2.93  | 7.0   | 1.97  |
| Analytical results:                                       |                 |       |       |       |       |       |       |       |       |
| (a) Fluoride (total)                                      | 4.0             | 5.2   | 4.3   | 6.0   | 0.5   | 0.35  | 2.5   | 0.35  | 0.25  |
| (b) Sulfate                                               | 1.10            | 0.83  | 1.10  | 0.63  | 1.95  | 1.95  | 1.97  | 1.95  | 1.33  |
| (c) Total fluoride-containing anion added (moles/liter)   | 0.172           | 0.073 | 0.093 | 0.100 | 0.057 | 0.059 | 0.036 | 0.133 | 0.007 |
| (d) Soluble fluoride-containing anion found (moles/liter) | 0.052           | 0.048 | 0.038 | 0.053 | 0.026 | 0.019 | 0.022 | 0.019 | 0.003 |

As shown in examples 5 and 6 of table I, an excess of cerous ion may be utilized to reduce or suppress the concentration of the fluoride ion as desired. Table I also illustrates that use of the complex fluoride provides a greater total fluoride content than the simple fluoride. It is to be noted that the catalytic ac-

70  
75  
over long periods of use and show that the oxidation of cerous ion to ceric ion apparently does not occur even after electrolysis for extended time periods as long as the bath is free of nitric ion or other catalytic oxidative ions. In addition, the results confirm the uniformity of electrodeposition characteristics

and prove that no substantial oxidation of cerous ion occurs, since oxidation of cerous ion to ceric ion would cause more undissolved cerous fluoride to go into solution and thus result in higher fluoride concentrations than were found on analysis.

Although this invention has been illustrated by reference to specific embodiments, modifications thereof which are clearly within the scope of the invention will be apparent to those skilled in the art.

I claim:

1. A process for electroplating chromium plate onto a basis metal which comprises passing current from an anode to a cathode at least a portion of which contains a conductive metal layer through an aqueous acidic chromium plating solution substantially free of nitric acid or other oxidative catalyst containing

1. at least one chromium compound providing hexavalent chromium ions for electroplating chromium; and

2. cerous ions in combination with fluoride ions or fluoride-containing complex ions and sulfate ions as catalysts; for a time sufficient to deposit a chromium electroplate having a thickness of at least  $1 \times 10^{-4}$  mm.

2. A process for electroplating chromium plate onto a basis metal as claimed in claim 1 wherein the aqueous acidic chromium-plating solution contains about 100-600 g./l. of chromic acid.

3. A process for electroplating chromium plate onto a basis metal as claimed in claim 1 wherein the electroplating process is carried out at 30°-70° C.

4. A process for electroplating chromium plate onto a basis metal as claimed in claim 1 wherein the aqueous acidic chromium plating solution contains about 100-600 g./l. of chromic acid and is saturated with a cerous salt at 30°-70° C.

5. A process for electroplating chromium plate onto a basis metal as claimed in claim 1 wherein the aqueous acidic chromium-plating solution contains about 100-600 g./l. of chromic acid and is saturated with CeF<sub>3</sub> at 30°-70° C.

6. A process for electroplating chromium plant onto a basis metal as claimed in claim 1 wherein the aqueous acidic

chromium-plating solution contains about 200-350 g./l. of chromic acid and 1-4 g./l. of CeF<sub>3</sub>.

7. A process for electroplating chromium plate onto a basis metal as claimed in claim 1 wherein the aqueous acidic chromium-plating solution contains about 200-400 g./l. of chromic acid, about 1-4 g./l. of cerous salt, and wherein the chromic acid to sulfate ion ratio is 100-550:1.

8. A composition for electroplating chromium plate onto a basis metal which is substantially free of oxidative catalyst which comprises

1. at least one chromium compound providing hexavalent chromium ions on aqueous media for electroplating chromium; and

2. cerous ions in combination with fluoride ions and sulfate ions as catalysts.

9. A composition for electroplating chromium plate onto a basis metal which is substantially free of oxidative catalyst as claimed in claim 8 wherein the concentration of chromic acid is about 100-600 g./l.

20 10. A composition for electroplating chromium plate onto a basis metal which is substantially free of oxidative catalyst as claimed in claim 8 wherein the concentration of chromic acid is about 200-350 g./l. and the composition for electroplating is saturated with a cerous salt at 30°-70° C.

25 11. A composition for electroplating chromium plate onto a basis metal which is substantially free of oxidative catalyst as claimed in claim 8 wherein the concentration of chromic acid is about 200-350 g./l. and the composition for electroplating is saturated with CeF<sub>3</sub> at 30°-70° C.

30 12. A composition for electroplating chromium plate onto a basis metal which is substantially free of oxidative catalyst as claimed in claim 8 wherein the concentration of chromic acid is 200-350 g./l. and the composition for electroplating contains 1-4 g./l. of CeF<sub>3</sub>.

35 13. A composition for electroplating chromium plate onto a basis metal which is substantially free of oxidative catalyst as claimed in claim 8 wherein the concentration of chromic acid is about 200-400 g./l., the chromic acid to sulfate ion ratio is 100-500:1 and the composition for electroplating contains about 1-4 g./l. of cerous salt.

\* \* \* \* \*